

## UNITED STATES PATENT OFFICE

2,179,151

## MOTOR FUEL

James W. Jean, Pasadena, Calif.

No Drawing. Application September 13, 1937,  
Serial No. 163,609

1 Claim. (Cl. 44—9).

The primary object of my invention is to provide a fuel compound that can be used satisfactorily as a substitute for gasoline or other hydrocarbon oil in internal combustion engines and for other industrial purposes, said compound possessing all of the desirable qualities of gasoline and other mineral hydrocarbon oils. My improved product is designed to be independent of mineral oil shortage, less expensive than hydrocarbon mineral oil fuel, and to utilize waste and low grade materials as a source of production.

In producing my improved motor fuel, I employ raw ingredients, such as corn, corn cobs, corn stalks, table refuse, spoiled crops, wood saw dust, wood chips, wood shavings, cellulose, wheat, rye, oats, barley, rice, beet roots, potatoes, peanut hulls, horse chestnuts, and waste and fermented products which are entirely free from coal tar or petroleum derivatives. These products are reduced by fermentation and distillation to butyl alcohol, acetone, ethyl ether, anhydrous ethyl alcohol and vegetable oil, or by chemical synthesis from chemicals and gases procured solely from said ingredients. Certain of these resultant ingredients may be mixed in proper proportions as hereinafter set forth and the resulting liquid is a motor fuel which will vaporize and when compressed in an internal combustion engine, will readily ignite and explode. I have found that the following ingredients produced as stated above and assembled in substantially the following proportions will produce a highly efficient and effective motor fuel:

|                                                   | Per cent |
|---------------------------------------------------|----------|
| 35 (N) Butyl alcohol                              | 38       |
| (95%) Ethyl alcohol or (ethyl or sulphuric ether) | 10       |
| Acetone                                           | 30       |
| Turpentine or (toluol)                            | 4        |
| 40 Benzol                                         | 18       |

These ingredients are thoroughly mixed together and are then ready for use. I have found that this combination of ingredients has marked advantages as a motor fuel, among which are the following:

The operation of an internal combustion engine using my improved fuel is smooth, while power put-put is good and fuel consumption low; substantially no carburetor adjustment is required beyond that used for carbureting gasoline; practically no carbon deposit occurs upon the

inner surfaces of the cylinder, piston head and valves; no carbon knock occurs, and the engine produces good heavy pulling characteristics with substantially no overheating effect. My improved fuel compound can be readily compressed to a highly efficient extent, has a high flash test, is permanent and will not separate into constituent parts after long standing or being subjected to ordinary changes of temperature, is substantially completely consumed by combustion when used, is more economical than most other fuels when used to operate internal combustion engines, and may be used in place of gasoline and other fuel oil most effectively.

The proportions of ingredients used may be varied substantially 5% either way to suit varied conditions. Also up to 8% of ethyl or sulphuric ether may be added to replace an equal amount of ethyl alcohol or acetone for easier starting of the motor and to increase vapor pressure.

Primarily the butyl alcohol provides power accompanied by high volatility to the product. The ethyl alcohol and acetone increase the vapor pressure and make starting in cold weather easier. The turpentine (or toluol) is used to increase the air fuel ratio and to insure the proper heat content. The benzol increases the air fuel and acts as a stabilizer as well as to increase the heat content. As the butyl alcohol and ethyl alcohol normally do not have the proper amount of heat units to compare with the type of fuel being used in present day equipment and require a lower air fuel ratio, it is desirable to substitute the ethyl alcohol, acetone, turpentine, ether and benzol in varying proportions as stated so as to build up the heat units as well as to increase the vapor pressure.

I have stated generally the ingredients and proportions thereof of which my improved fuel may be composed but I desire to have it understood that the ingredients may, within the doctrine of equivalents be varied in proportion and otherwise, within the scope of the following claim.

I claim:

A fuel, employing a mixture of ingredients fermented and distilled from fermentable products, consisting of butyl alcohol 38 parts, ethyl alcohol 10 parts, acetone 30 parts, turpentine 4 parts and benzol 18 parts.

JAMES W. JEAN.

50